

Patented Apr. 24, 1928.

1,667,083

## UNITED STATES PATENT OFFICE.

ROSCOE B. SMITH, OF KENVIL, NEW JERSEY, AND ERNEST M. SYMMES, OF WILMINGTON, DELAWARE, ASSIGNEES TO HERCULES POWDER COMPANY, OF WILMINGTON, DELAWARE, A CORPORATION OF DELAWARE.

## GELATIN-DYNAMITE EXPLOSIVE.

No Drawing.

Application filed November 27, 1926. Serial No. 151,243.

For many years the lowest strength of their surface, we afford a continuous film 55 on which the wave of detonation can travel throughout the mass. By a study of the individual absorbencies of the ingredients other than the explosive ingredients we have determined just which non-explosive ingredients, and in what proportion of each, should be used to absorb as a surface film the liquid explosives employed. The non-explosive ingredients that we have added have the characteristic that they do not subsequently, with time, absorb into their mass the liquid explosive, but merely retain the latter on their surface. This facilitates the passage of the wave of detonation through the mass and so maintains indefinitely the 70 sensitiveness to detonation.

|                              | Per cent. |
|------------------------------|-----------|
| 5 Nitroglycerin, etc-----    | 31        |
| Nitrocompounds-----          | 2         |
| Nitrocotton-----             | 0.6       |
| Sodium nitrate-----          | 52.7      |
| 10 Wood pulp-----            | 2.2       |
| Corn meal or ivory meal----- | 4.5       |
| Flour or corn starch-----    | 3.0       |
| Sulphur-----                 | 3.0       |
| Chalk-----                   | 1.0       |
| 15                           | 100.0     |

By successive steps the strength was reduced by cutting down the nitroglycerin content until in later years a so-called twenty-five per cent gelatin dynamite was successfully produced. This comprised:

|                              | Per cent. |
|------------------------------|-----------|
| Nitroglycerin, etc-----      | 23.5      |
| Nitrocompounds-----          | 1.5       |
| 25 Nitrocotton-----          | 0.3       |
| Sodium nitrate-----          | 59.0      |
| Corn meal or ivory meal----- | 2.5       |
| Flour or corn starch-----    | 2.5       |
| Sulphur-----                 | 9.7       |
| 30 Chalk-----                | 1.0       |
|                              | 100.0     |

Such a twenty-five per cent gelatin dynamite was considered as low a strength as could be obtained, because if the nitroglycerin content were lowered still further the mixture would be too dry and stiff to be satisfactory as a gelatin dynamite, could not be packed into shells by any practical machines, and would have an unsatisfactorily low sensitiveness to detonation.

We have discovered that by still further reducing the nitroglycerin content but simultaneously adding more of a liquid of low explosive strength, such as liquid dinitrotoluol, the explosive strength of a gelatin may be reduced to a 20% strength while still leaving sufficient liquid present to avoid the above mentioned difficulty of too dry, stiff and insensitive a gelatin. We have also discovered that by using non-absorbent carbonaceous materials, which merely retain the gelatinized nitroglycerin-dinitrotoluol mixture on

|                           | Per cent. |
|---------------------------|-----------|
| Nitroglycerin, etc-----   | 18        |
| Liquid dinitrotoluol----- | 4         |
| Nitrocotton-----          | .2        |
| Sodium nitrate-----       | 63.3      |
| Sulphur-----              | 9         |
| 20 Starch-----            | 3.3       |
| Ivory meal-----           | 1.2       |
| Chalk-----                | 1         |
| 30                        | 100.0     |

This composition has a sensitiveness of 6-8", a strength of a 20% gelatin dynamite, and works easily through the usual type of packing machines; and since the non-explosive ingredients are non-absorbent, the explosive ingredients are not absorbed into the mass of the non-explosive ingredients.

The percentage of nitroglycerine should not much exceed eighteen per cent, but may be as low as about seventeen per cent. The percentages of liquid dinitrotoluol and nitrocotton should not materially exceed the percentages specified in the example composition, although the proportion of each may be reduced fifty per cent below the percentages specified. The percentage of sodium nitrate may vary from sixty to sixty-five per cent. The percentage of sulphur should not be substantially below that specified in the example composition, but may be increased to twelve per cent. The percentages of starch and ivory meal are variable within wide limits. Ivory meal may constitute as

much as two per cent of the composition, but it may be omitted although. In general, the smaller the proportion of ivory meal, the larger should be the proportion of starch, 5 which may, therefore, have a permissible percentage range of from two to five per cent. The percentage of chalk should not vary materially from that specified in the example composition.

10 It will be understood that in specifying liquid dinitrotoluol as one of the ingredients of the explosive, it is not intended to exclude known equivalents, of which trinitrotoluol is an example. Potassium nitrate may be substituted for sodium nitrate, but with added 15 cost and without any compensating advantage. For starch may be substituted corn flour.

It is well known that in the manufacture 20 of gelatin dynamites, any of the well known nitroglycerines may be employed; for example, trinitroglycerine, tetranitrodiglycerine, dinitrochlorhydrene, dinitroglycol, nitrohydrene, or combinations of any two or 25 more of them.

It will be understood that in the claims where specific substances are set forth, it is not intended to exclude the use in place thereof of known equivalents, of which examples are herein given. 30

Having now fully described our invention, what we claim and desire to protect by Letters Patent is:

A low strength dynamite explosive comprising the below specified ingredients each 35 within the proportion range specified, namely, nitroglycerin, 17-18 per cent; dinitrotoluol, 2-4 per cent; nitrocotton, .1-.2 per cent; sodium nitrate, 60-65 per cent; sulphur, 9-12 per cent; starch 2-5 per cent; 40 and a small proportion of chalk.

In testimony of which invention, I, ROSCOE B. SMITH, have hereunto set my hand at Kenvil, N. J., on this 23rd day of November, 1926, and I, ERNEST M. SYMMES, have 45 hereunto set my hand at Wilmington, Delaware, on this 24th day of November, 1926.

ROSCOE B. SMITH.  
ERNEST M. SYMMES.